

June 4, 1957

KEIZO IWASE ET AL

2,794,731

## METHOD OF REDUCING REFINING OF CAST IRONS AND STEELS

Filed July 21, 1954



Fig 1



Fig 2



Photo. 1

$\times 100$   
no etched



Photo. 2

$\times 100$   
nital etched



Photo.3

$\times 100$   
nitro etched

2,794,731

## METHOD OF REDUCING REFINING OF CAST IRONS AND STEELS

Keizo Iwase and Masao Honma, Sendai City, Japan, assignors to The Research Institute for Iron, Steel and Other Metals of The Tohoku University, Sendai City, Japan

Application July 21, 1954, Serial No. 444,694

2 Claims. (Cl. 75—57)

This invention relates to a method of reducing refining of cast irons and steels.

The principal object of this invention is to produce

jecting the molten metal after tapping to inoculation with ferro-silicon.

According to the characteristic features of this invention, a cast iron melt is subjected to the reducing refining with use of a reducing slag as described hereinafter in a melting furnace such as an electric arc furnace, high frequency induction furnace, crucible furnace, heavy oil furnace and the like, and then the tapped molten metal may or may not be treated with ferro-silicon, calcium silicide and the like for inoculation, thus it enables to produce cast iron having properties comparable with superheated cupola cast iron inoculated by calcium silicide or magnesium treated nodular cast iron.

After fundamental investigations, the inventors have found out that there exists such relations as listed in the following table between various properties of cast iron and oxygen content dissolved in the cast iron melt:

TABLE  
*Relation between oxygen content and various properties of cast iron.*

| Dissolved Oxygen                | Decreased ← → Increased                                     |                             |                                                                 |                                                  |                              |                                                       |                           |                               |                      |                                        |
|---------------------------------|-------------------------------------------------------------|-----------------------------|-----------------------------------------------------------------|--------------------------------------------------|------------------------------|-------------------------------------------------------|---------------------------|-------------------------------|----------------------|----------------------------------------|
|                                 | VI'                                                         | V                           | IV'                                                             | III'                                             | II'                          | I                                                     | II                        | III                           | IV                   | V                                      |
| Macro Structure (10-30m/m Cast) | White                                                       | Inverse Chilled             | Grey                                                            | Grey                                             | Grey                         | Grey                                                  | Grey                      | Grey                          | Inverse Chilled      | White                                  |
| Graphite and Matrix             | Needle like eutectic Fe <sub>3</sub> C and nodular graphite | Outer IV'<br>Inner VI'      | Fine Granular graphite<br>Ferrite                               | Eutectic graphite<br>Pearlite                    | Rose graphite<br>Pearlite    | Flake graphite<br>Pearlite                            | Rose graphite<br>Pearlite | Eutectic graphite<br>Pearlite | Outer III<br>Inner V | Ledeburitic eutectic Fe <sub>3</sub> C |
| Strength                        |                                                             |                             |                                                                 |                                                  |                              |                                                       |                           |                               |                      |                                        |
| Toughness                       |                                                             |                             |                                                                 |                                                  |                              |                                                       |                           |                               |                      |                                        |
| Mass Effect                     |                                                             |                             |                                                                 |                                                  |                              |                                                       |                           |                               |                      |                                        |
| Variety of Cast Iron            | Mg Treated Nodular Cast Iron                                | Cast Iron of this invention | Super-heated Cupola Cast Iron<br>inoculated by Calcium Silicide | Super-heated Cupola Cast Iron<br>by Charcoal Pig | Cupola Cast Iron by Coke Pig | Acidic Electric Cast Iron<br>Basic Electric Cast Iron |                           |                               |                      |                                        |

It will be seen from the above that strength decreases from a maximum for a minimum of dissolved oxygen to reach a low point at I and thereafter increases with increasing oxy-

gen. Toughness decreases continuously without intermediate low point, and Mass Effect increases continuously with increasing oxygen.

splendid cast iron which is comparable with the highest grade cast iron obtainable at present.

A further object of this invention is to improve the quality of steel by the reducing refining.

It is known that super-heated cupola cast iron inoculated by calcium silicide and nodular cast iron treated with magnesium has a very high tensile strength. Cast iron having such high tensile strength as super-heated cupola cast iron inoculated by calcium silicide and magnesium treated nodular cast iron could never be obtained until at present by reducing refining in a melting furnace such for example as an electric arc furnace, high frequency induction furnace, crucible furnace by means of slag such as white slag, carbide slag, etc., and by sub-

Electric furnace cast iron obtained by using heretofore common white slag or carbide slag has an oxygen content in the range within II, III and IV in the above table. Such electric furnace cast iron is usually deficient in toughness, and contains unevenly distributed graphite of smaller size, and has poor fluidity. It is known that these are mainly due to a larger oxygen content.

Cast iron obtainable by this invention has an oxygen content in the ranges within II' to V' and shows particularly superior quality if subjected to inoculation treatment. Deoxidized cast iron melt within the range of III' to V' is preferably inoculated. If not inoculated, graphite is finer due to the super-cooling of the melt. The graphite takes eutectic, fine granular, short-flake, quasi-

flake or nodular form in the structure according to the degree of deoxidation and inoculation.

According to this invention, the inventors have accomplished an epochmaking discovery, based on the fundamental theory which they have established relating to the reducing slags which can develop much stronger reducing effect than heretofore used white slag and carbide slag, and the art of producing such slags. By the reducing refining of cast iron melt with a slag according to this invention, a very strong and tough cast iron can be obtained, which is comparable or rather superior to known super-heated cupola cast iron inoculated by calcium silicide and magnesium treated nodular cast iron.

The slags which are found to be most suitable in carrying out this invention are ennumerated below:

(1) A mixture of one or more oxides or carbonates of the alkali or alkaline earth metals, and one or more of carbon, silicon (including silicon compounds such as ferro-silicon, and siliceous alloys) or aluminum (including aluminum alloys), and

(2) Calcium cyanamide containing  $\text{SiO}_2$ ,  $\text{Al}_2\text{O}_3$  or  $\text{CaO}$ .

Further in the economical point of view and considering the regulation of composition of slag to obtain a required reducing degree, basicity or acidity, a suitable amount of ordinary used other oxides such as  $\text{SiO}_2$ ,  $\text{Al}_2\text{O}_3$ ,  $\text{MgO}$  etc., carbonates, or slages such as blast furnace clag, cupola slag, open earth slag or electric furnace slag may be added to the above mentioned essential ingredients, and also the substance containing the above main slags as the main constituent may be used in this invention. Dolomite-C belongs to the reducing slag of this invention since it contains  $\text{CaCO}_3$ .  $\text{CaCN}_2$  sometimes contains considerably small amount of reactive calcium as the result of weathering so that it is advantageous to add C, Si and Al to  $\text{CaCN}_2$ , then it will become a slag such as  $\text{CaO-C-CaCN}_2$  which also constitutes a reducing slag in accordance with this invention.

Some examples of compositions of the reducing slag which is the characteristic feature of this invention are as follows:  $\text{BaCO}_3\text{-C}$ ;  $\text{Na}_2\text{CO}_3\text{-C}$ ;  $\text{Na}_2\text{CO}_3\text{-BaCO}_3\text{-C}$ ;  $\text{CaCO}_3\text{-C}$ ;  $\text{CAO-C}$ ;  $\text{BaCO}_3\text{-Si}$ ;  $\text{BaCO}_3\text{-C-Si}$ ;  $\text{BaCO}_3\text{-Al}$ ;  $\text{BaCO}_3\text{-Si-Al}$ ;  $\text{SrO-C}$ ;  $\text{SrCO}_3\text{-C-Al}$ ; ordinary slag (for example  $\text{CaO-SiO}_2\text{-Al}_2\text{O}_3$ )- $\text{CaCN}_2$ ;  $\text{CaO-CaCN}_2$ ;  $\text{CaO-CaCN}_2\text{-C}$ .

In carrying out the method of this invention, about 1 to 15% of the above slag may be added to raw metal material of suitable constituents and the reducing refining can be conducted, for example, in an electric arc furnace or a high frequency induction furnace. Although it is a particular advantage that the slag can be reacted at a sufficiently low temperature within the range of about  $1300^\circ\text{C}$ . to  $1350^\circ\text{C}$ ., yet the reducing refining may be promoted at a higher temperature so that the use of electric arc furnace is more preferable. It is not necessary to maintain reducing atmosphere in the furnace specially in carrying out the reducing refining according to this invention. Though a basic furnace is preferable, yet an acidic furnace may also be used without objection.

According to this invention, it is necessary that in the method of preparing the slag, each part of the reducing slag is reactive with slag constituents, before the slag is added with the raw metal material to be refined by reduction. The art of preparing slag is one of the most important points because the object of this invention could never be obtained by merely charging the above mentioned slag constituents into a melting furnace.

The electric furnace cast iron obtainable with use of white slag or carbide slag for reducing refining is usually brittle, less fluidity, liable to chill, larger mass effect and poor castability, and the inventors have found the fact that such defects are due to the imperfect art of preparing slag. Cast iron produced according to this invention has higher tensile strength and larger deflection, and considerably good fluidity and castability without substantially mass effect, and the cast iron of low carbon and sili-

con amounts which should invariably become white cast iron by heretofore usual smelting process, enables to produce grey cast iron instead of white cast iron by the method of this invention.

The fundamental difference between the method of this invention and the heretofore usual melting process in an electric furnace and cupola will be evident from the following comparison:

1. In the present method, the reducing slag is independent of its form whether it is in the liquid state or solid state. Accordingly the mixture of reducing slag of solid state having such a composition as to have higher melting point than that of cast iron may be arranged on the side wall and bottom surface of the melting furnace and the reducing refining is carried on from the surrounding surface of molten metal by charging the reducing slag, thereby resulting the most effective reducing refining of a larger amount of molten metal in a given time. Such process has never been tried before and the method of this invention enables to use a cupola or reverberatory furnace for the melting purpose.

2. According to the present method, lathe chips or turning scrap of cast iron or steel may be used as raw material with high yield of the required cast iron.

3. On the other hand, in known methods of producing super-heated cupola cast iron inoculated by calcium silicide, which is of the highest quality, selected steel scrap should be used as the raw material, but coke pig iron could never be used. The production of magnesium treated nodular cast iron also needs special high grade raw material.

According to this invention, a large amount of coke pig iron may be used as raw material to obtain a cast iron having the tensile strength of 41 to 42 kg./mm.<sup>2</sup> and the structure in the form of uniformly dispersed short-flake graphite and sorbitic pearlite, and also a cast iron having tensile strength of about 60 kg./mm.<sup>2</sup> containing substantially no free cementite and having the structure of nodular graphite and sorbitic pearlite. Creation of dense pearlite is due to the lowering of  $\text{Ar}_1$  by the strong deoxidation.

4. According to the present method, the reducing refining can be conducted at a lower melting temperature such as about  $1300^\circ\text{C}$ . to about  $1350^\circ\text{C}$ ., and enables to obtain the above described eutectic graphite cast iron (III'), fine granular graphite cast iron (IV') and nodular graphite cast iron (VI').

In contradistinction to the above, the heretofore known method of reducing refining using white slag or carbide slag could neither be conducted at such a low temperature nor considered its possibility. The properties of cast iron deoxidized within the range of (II') to (IV') corresponds with those of cast iron which was melted in a cupola under super-heated condition and tapped at a temperature above about  $1550^\circ\text{C}$ . Thus the cast iron obtained from a melting furnace by the method of this invention without subjecting inoculation treatment after it has been tapped out of the furnace may have the properties similar to those of super-heated cupola cast iron so that it should be noted that such non-inoculated cast iron should come within the scope of this invention.

5. The least amount of carbon and silicon which a plain cast iron heretofore produced in an electric furnace by reducing refining with use of white slag or carbide slag would become grey cast iron, not becoming white cast iron or mottled cast iron, are 3.3 to 3.5% of C and about 1.5% of Si for a test piece made in a green sand mold having 10 mm. in diameter.

On the other hand, the plain cast iron obtained by the method of this invention in a green sand mold of 10 mm. diameter does not contain free  $\text{Fe}_3\text{C}$  at the condition of C and Si such, for instance, as 3.00% C and 0.97% Si; 2.43% C and 0.69% Si; 1.96% C and 1.10% Si; and 1.62% C and 2.29% Si respectively and consists of graphite and pearlite matrix.

The method of this invention also can be applied to the

smelting of ferro-alloys such as silicon steel and other steels for the purpose of strong deoxidation, thereby improving the various properties of silicon steel and increasing self-hardening effect of steel since its pearlitic lamellar becomes sorbitic lamellar due to the lowering of the  $A_1$  point.

The annexed drawings show the properties of cast iron obtainable by the method of this invention, in which

Figs. 1 and 2 are diagrams showing the mass effect of two test pieces made by the method of this invention, and

Photo. Nos. 1 to 3 show structure of the test pieces made by the method of this invention.

Some examples of this invention are shown in the following:

#### Example I

*Raw metal materials.*—Blast furnace coke pig iron, returned ordinary cast iron such as gate and risers etc., lathe chips, steel scrap etc.

*Melting process.*—Héroult electric furnace, or high frequency induction furnace.

The reducing refining is conducted according to the method of this invention using, for example, the following slags:

- (i) In which the ratio of  $BaCO_3$  to C is 5 to 1
- (ii) In which the ratio of  $CaO$  to  $CaCN_2$  is 1 to 1
- (iii) In which the ratio of  $CaCO_3$  to C is 5 to 1

Any one of the above slags gave the same result.

After tapping, the melt was inoculated with about 0.05% ferro-silicon.

*Result.*—Chemical compositions, mechanical properties and mass effect are as follows:

|            |         |        |
|------------|---------|--------|
| Total C    | percent | 3.40.  |
| Graphite C | do      | 2.70.  |
| Combined C | do      | 0.70.  |
| Si         | do      | 1.49.  |
| Mn         | do      | 0.51.  |
| P          | do      | 0.128. |
| S          | do      | 0.009. |

#### Tensile strength test:

|                                              |                             |
|----------------------------------------------|-----------------------------|
| Mold                                         | 30 mm. diameter.            |
| Test piece                                   | 20 mm. diameter.            |
| Length of parallel portion of the test piece | 25 mm.                      |
| Load                                         | 9.5 tons.                   |
| Tensile strength                             | 30.2 kg./mm. <sup>2</sup> . |

#### Transverse strength testing:

|                           |                  |
|---------------------------|------------------|
| Mold                      | 37 mm. diameter. |
| Test piece                | 30 mm. diameter. |
| Distance between supports | 300 mm.          |
| Load                      | 2.1 tons.        |
| Deflection                | 4.5 mm.          |

The structure consists of eutectic or fine granular graphite and sorbitic pearlitic matrix.

The mass effect was measured by the Brinell hardness numbers at a cross-section through the central position of a K-shaped test piece 300 mm. long as shown in Fig. 1 and it was found that there is substantially no mass effect.

*Remark.*—Electric furnace cast iron produced in a basic Héroult furnace with white slag or carbide slag according to heretofore ordinary method has tensile strength of about 25 kg./mm.<sup>2</sup> and deflection of about 2.0 mm, and the mass effect is considerably larger than that of a cast iron obtainable by the method of this invention.

#### Example II

*Raw metal materials.*—Same as Example I.

*Process for melting.*—Same as Example I.

Melt after tapping was inoculated with about 0.2% ferro-silicon.

*Results.*—Results of chemical composition, mechanical strength and mass effect are as follows:

|                                                 |                      |       |
|-------------------------------------------------|----------------------|-------|
| Total C                                         | percent              | 2.9   |
| Si                                              | do                   | 0.75  |
| Mn                                              | do                   | 0.52  |
| P                                               | do                   | 0.03  |
| S                                               | do                   | 0.008 |
| Tensile strength (test piece same as Example I) | kg./mm. <sup>2</sup> | 42.33 |
| Deflection (test piece same as Example I)       | mm                   | 10.0  |

The mass effect was shown by the Brinell hardness number tested on the cross-sectional surface cut through the middle of a cube of 20 cm. as shown in Fig. 2, and it was found that every point showed almost equal hardness and the mass effect is very small.

The structure is shown by Photo. No. 1 (37 mm. diameter, cast) and consists of uniformly dispersed short-flaked graphite and sorbitic pearlite.

*Remark.*—Electric furnace cast iron reducing refined with heretofore method using white slag or carbide slag, even after it was inoculated with ferro-silicon, will become white cast iron or mottled cast iron with the composition shown in this example.

#### Example III

*Raw metal material.*—Same as Example I.

*Process of melting.*—Same as Example II.

*Results.*—Results of chemical composition, mechanical properties and mass effect are as follows:

|                                                 |                      |         |
|-------------------------------------------------|----------------------|---------|
| Total C                                         | percent              | 1.63    |
| Si                                              | do                   | 2.80    |
| Mn                                              | do                   | 0.74    |
| P                                               | do                   | 0.03    |
| S                                               | do                   | 0.007   |
| Tensile strength (test piece same as Example I) | kg./mm. <sup>2</sup> | 62.3    |
| Elongation                                      | percent              | 2.5-5.0 |
| Tensile strength after short time annealing     | kg./mm. <sup>2</sup> | 55.2    |
| Elongation                                      | percent              | 14.3    |

The structure, under the cast state, is shown by Photo. No. 2 and consists of nodular graphite ferrite and sorbitic pearlite with no free  $Fe_3C$ . The structure after short time annealing is shown by the Photo. No. 3, consisting of annealed graphite and ferrite.

By adjusting the amounts of C and Si, a structure consisting of nodular graphite and ferrite under the cast state may be obtained.

*Remark.*—Electric furnace cast iron produced by heretofore ordinary reducing refining method using white slag or carbide slag, even after inoculated with ferro-silicon, is white cast iron or mottled cast iron with the chemical composition in this example.

What we claim is:

1. A method of producing tough cast iron and steel containing short flake graphite and nodular graphite which comprises reducing-refining the raw metal in a melting furnace with a refining agent containing a substance selected from the group consisting of the oxides and carbonates of the alkali and alkaline earth metals and a substance selected from the group consisting of carbon, silicon and aluminum and a further refining agent comprising  $CaCN_2$  and a substance selected from the group consisting of  $SiO_2$ ,  $CaO$  and  $Al_2O_3$ .

2. A method of producing tough cast iron and steel containing short flake graphite and nodular graphite which comprises reducing-refining the raw metal in a melting furnace with a refining agent comprising a substance selected from the group consisting of the oxides and carbonates of the alkali and alkaline earth metals and a substance selected from the group consisting of

carbon, silicon and aluminum and a further refining agent comprising  $\text{CaCN}_2$  and  $\text{SiO}_2$ .

References Cited in the file of this patent

UNITED STATES PATENTS

1,335,370 Ellis ----- Mar. 30, 1920  
2,606,112 Jordan ----- Aug. 5, 1952

699,495  
702,776

FOREIGN PATENTS

Great Britain ----- Nov. 11, 1953  
Great Britain ----- Jan. 20, 1954

OTHER REFERENCES

"Refining Metals Electrically," 1st ed., pages 268 to 272, inclusive. Edited by Barton. Published in 1926 by The Penton Publishing Co., Cleveland, Ohio.